

# UNITED STATES PATENT OFFICE.

NATHAN BOOTH, OF ALEXANDRIA, INDIANA, ASSIGNOR TO BANNER ROCK PRODUCTS COMPANY, OF ALEXANDRIA, INDIANA, A CORPORATION OF INDIANA.

## INSULATING COMPOUND.

No. 884,456.

Specification of Letters Patent.

Patented April 14, 1908.

Application filed April 20, 1907. Serial No. 369,342.

*To all whom it may concern:*

Be it known that I, NATHAN BOOTH, a citizen of the United States, residing at Alexandria, in the county of Madison and State of Indiana, have invented certain new and useful Improvements in Insulating Compounds, of which the following is a specification.

The object of my invention is to provide a composition, preferably in the form of plates or boards, which shall be both water-proof and a good heat insulator whereby the plates or boards are especially adapted for use for walls, partitions and floors in cold storage houses, etc.

My invention, in its entirety, consists of a plate or board formed of a composition of mineral in fibrous form (as for instance mineral or rock wool, asbestos, etc.), peat (preferably thoroughly decomposed), wood pulp, flour or other gluten, and a sufficient quantity of grease thoroughly impregnating the entire mass. The peat should be of a mucky or fibrous nature, such as is found in bogs, and I designate such peat as bog peat.

In practice I have a desirable product in the following manner: I first produce a binder consisting of approximately 25 per cent. peat, 25 per cent. wood pulp, 37 per cent. grease (which may be either animal fat, petroleum or other grease) and 13 per cent. flour. The proportions may be varied somewhat without deleterious results. This binder is conveniently formed by thoroughly disintegrating the peat in a sufficient quantity of water to make a thick mush and associating the wood pulp, grease and flour therewith. I have found that the peat itself is a very good binder for the fibrous mineral and that it seems to have a decided affinity for the grease so that it is entirely possible to make a thorough mixture of the grease and peat as well as the wood pulp and gluten even in the presence of a considerable quantity of water.

The mineral fiber is placed in water and

agitated by any desired means until the fibers are properly separated and I then associate with the fiber from 15 to 20 per cent., more or less, of the binder already described. The grease having become thoroughly associated with the binder it does not separate therefrom when the binder is placed in the water with the fibers but, by proper agitation, the binder becomes thoroughly mixed with the mineral fiber. Thereupon the water is drawn off and the mass formed, in any desired manner, into desirable shapes. As soon as the water is drawn off the grease is able to permeate the entire mass quite uniformly and thus render the product water-proof. By this process I am able to obtain a thorough permeation and water-proofing of the articles with a much smaller proportion of grease than would be required if an attempt were made to permeate the articles with the grease after the articles have been formed.

I claim as my invention:

1. A composition of matter comprising mineral fibers, peat and grease.

2. A composition of matter comprising mineral fibers, peat, wood pulp, flour or other gluten and grease.

3. A composition of matter comprising mineral fibers, bound together with a binder comprising peat, wood pulp, grease and gluten.

4. A composition of matter comprising mineral fibers bound together with a binder comprising approximately 25 per cent. peat, 25 per cent. wood pulp, 37 per cent. grease and 13 per cent. flour or other gluten.

In witness whereof, I, have hereunto set my hand and seal at Alexandria, Indiana, this sixteenth day of April, A. D. one thousand nine hundred and seven.

NATHAN BOOTH. [L. S.]

Witnesses:

JAMES S. WALES,  
HORACE J. INLON.